

## 1

2,829,091

## METHOD FOR ELECTROPLATING TITANIUM

Leo Missel, North Hollywood, Calif., assignor to Menasco Manufacturing Company, Burbank, Calif., a corporation of California

No Drawing. Application June 4, 1956  
Serial No. 588,972

9 Claims. (Cl. 204—32)

This invention relates to the metal coating art, and has particular reference to a process and composition for treating the surfaces of titanium and titanium alloys to permit subsequent treatment, such as electroplating, of the same.

Titanium and titanium alloys are finding increasing uses and applications, particularly in the aircraft industry, due primarily to the excellent strength-weight ratios of the metal and its alloys. However, these materials exhibit tendencies toward galling, seizing and excessive wear when utilized in applications requiring motion between components such as in bearings, sliding assemblies and the like.

One of the principal objects of this invention is, therefore, to provide a process for the treatment of titanium and its alloys to permit the application thereto of a hard metal coating having satisfactory bearing characteristics.

Another object of this invention is to provide a process for the treatment of surfaces of titanium and titanium alloys to permit the electroplating thereon of metallic films having characteristics of adhesion, hardness, electrical conductivity, solderability, etc., comparable to films produced on common metals by conventional methods.

Another object of this invention is to provide a process for chromium plating the surfaces of titanium and titanium alloys.

Another object of this invention is to provide a process for chromium plating many different types of titanium alloys.

Other objects and advantages of this invention, it is believed, will be readily apparent from the following detailed description of preferred embodiments thereof.

Briefly, this invention includes the discovery that articles of titanium and titanium alloys may be treated with aqueous solutions of mixtures of hydrofluoric acid and chromic acid or its salts to render the surfaces of the articles receptive to subsequent electrolytic plating thereof to produce an adherent plate of chromium or other metals.

The following are specific examples of processes and compositions embodying the present invention, but it is to be understood that it is not intended to limit the invention to the specific steps set forth therein.

*Example 1*

Parts forged of a titanium alloy containing 4% aluminum and 4% manganese were cleaned with a conventional degreasing agent, rinsed and then immersed in an acid etch bath consisting of three parts by volume of 69% nitric acid and one part by volume of 60% hydrofluoric acid for a sufficient length of time at room temperature to chemically clean and activate the titanium surface (about 1 minute). While best results are obtained with the described mixture, other acids such as sulfuric, hydrochloric mixed with hydrofluoric acid, or hydrofluoric acid alone may be used.

The next step was to rinse the parts from the acid cleaning bath with distilled water, and they were then dipped into a chemical treatment bath for a period of about 20 minutes, the temperature of the bath being maintained at about 190° F. The bath comprised an

## 2

aqueous (distilled water) solution of the following ingredients in the proportions indicated:

*Example 1a*

5 Hydrofluoric acid (60% HF) \_\_\_\_\_ ml./liter 50  
Sodium dichromate (Na<sub>2</sub>Cr<sub>2</sub>O<sub>7</sub>.2H<sub>2</sub>O) \_\_\_\_\_ gm./liter 250

The parts were removed from this bath and rinsed thoroughly in cold running tap water. The parts were then chromium plated in a conventional hard chrome electroplating bath at 3 amperes per square inch for 4 hours, the bath temperature being maintained at 130° F. The plating solution consisted of 33 oz./gal. of chromic acid and 0.33 oz./gal. of sulfate ion.

15

20

The identical process and alloy of Example 1 and the treatment bath of Example 1a were utilized in copper plating the alloy in a copper sulfate bath (30 oz. CuSO<sub>4</sub> and 7 oz. H<sub>2</sub>SO<sub>4</sub> per gallon) at room temperature.

*Example 1b*

The identical process of Example 1 and the treatment bath of Example 1a were utilized in chrome plating parts of a titanium alloy containing 6% aluminum and 4% vanadium.

*Example 2*

The identical process of Example 1 and the treatment bath of Example 1a were utilized in chrome plating parts of a titanium alloy containing 5% chromium and 3% aluminum.

*Example 3*

The identical process of Example 1 and the treatment bath of Example 3a below were utilized in chrome plating parts of a titanium alloy containing 5% chromium and 3% aluminum.

30

35

Hydrofluoric acid (60% HF) \_\_\_\_\_ ml./liter 25  
Sodium dichromate (Na<sub>2</sub>Cr<sub>2</sub>O<sub>7</sub>.2H<sub>2</sub>O) \_\_\_\_\_ gm./liter 400

The bath of Example 3a comprised an aqueous (distilled water) solution of the above ingredients.

Excellent plating results were obtained with the process of the above examples. The adherence of the chromium plate under steel ball indentation tests and under specially designed bearing load tests was excellent and qualified the parts for use in heavy duty aircraft landing gear assemblies.

45 The chemical reactions and/or physical phenomena involved in the treatment with the chemical treatment bath of Example 1a are not entirely understood. It would appear, however, that the hydrofluoric acid in the bath plays an important part in the complete removal of the oxide film. It should be noted that the hydrofluoric acid may be formed in situ by the addition of a water-soluble salt of hydrofluoric acid and another acid, such as for example, sulfuric, hydrochloric, phosphoric, citric, etc.

50 The inclusion of the dichromate in the composition of Example 1a is also an important feature of the invention. It has been found that the dichromate makes possible a chromium plate which meets the requirements for heavily-loaded bearing surfaces. It is believed that this is due, in part at least, to the fact that the dichromate, in conjunction with the hydrofluoric acid, activates, or renders reactive, the titanium or titanium alloy surface. Although somewhat less satisfactory, other chromium compounds, such as, for example: chromic acid; alkali metal salts of a chromic acid such as sodium chromates, potassium and ammonium chromates and dichromates, and the hydrates of these compounds; and other water-soluble salts of a chromic acid may be substituted for, or admixed with, the sodium dichromate of Example 1a.

55 For obtaining maximum adherence, the concentration of the chromic compound in the treatment solution is critical and should be maintained above about 15% by weight. Optimum results with the alloy of Example 1

were obtained utilizing concentrations of sodium dichromate from 200 gm./liter to 400 gm./liter at a 60% hydrofluoric acid concentration of 50 ml./liter. At a dichromate concentration of 250 gm./liter, 60% hydrofluoric acid concentration of 25 ml./liter to 75 ml./liter gave excellent chrome plate adhesion with a 20-minute immersion time, and concentrations of 37.5 ml./liter to 62.5 ml./liter of 60% hydrofluoric acid gave excellent adhesion with a 10-minute immersion time.

With the alloy of Example 2, concentrations of 200 to 300 gm./liter of sodium dichromate and 50 ml./liter of 60% hydrofluoric acid at 10 and 20-minute immersion times gave excellent results. At a dichromate concentration of 200 gm./liter, 35 to 60 ml./liter of 60% hydrofluoric acid gave excellent results with a 20-minute immersion, while at 10 minutes, the hydrofluoric acid range was extended to 25 to 60 ml./liter.

With the alloy of Example 3, excellent results were obtained utilizing somewhat higher concentrations of sodium dichromate and lower concentrations of hydrofluoric acid. At a level of 400 gm./liter of dichromate, adherent chromium plate was obtained with 15-35 ml./liter of 60% hydrofluoric acid under immersion times of 10 and 20 minutes.

As indicated above, the proportions of the ingredients of Examples 1a and 3a may be varied, depending primarily upon the type of alloy and the treating time, and the relative proportions of the two ingredients. From a standpoint of commercial practicability, the concentration ranges are approximately as follows:

|                                      |                                      |
|--------------------------------------|--------------------------------------|
| Hydrofluoric acid                    | 0.5-20% (by weight as anhydrous HF). |
| Chromic acid or soluble salt thereof | 15% by weight to saturation point.   |
| Water                                | Balance.                             |

The temperature of the chemical treatment bath is preferably maintained within the range of about 180° to the boiling point, but lower temperatures, within reasonable limits, may be utilized. For best results at the temperatures indicated, the immersion time is at least five minutes, preferably from 10-20 minutes, and may be substantially longer.

It will be readily understood by those skilled in the art that the process and composition of this invention are not limited to the chromium plating operation. For example, parts treated as described may be given a copper plating from a conventional acid copper bath, or may be plated with any other conventional metal.

Having fully described my invention, it is to be understood that I do not wish to be limited to the details set forth, but my invention is of the full scope of the appended claims.

I claim:

1. A process for treating the surfaces of articles of titanium and titanium base alloys, including the steps of immersing said articles in a bath consisting essentially of an aqueous solution of 0.5% to about 20% by weight of hydrofluoric acid, and from about 15% by weight to the saturation point of a chromium compound selected from the group consisting of chromic acid and its salts, and electroplating said articles in a plating solution.

2. A process for treating the surfaces of articles of titanium and titanium base alloys, including the steps of immersing said articles in a bath consisting essentially of an aqueous solution of 0.5% to about 20% by weight of hydrofluoric acid, and from about 15% by weight to the saturation point of sodium dichromate, and electroplating said articles in a plating solution.

3. A process for treating the surfaces of articles of titanium and titanium base alloys, including the steps of immersing said articles in a bath consisting essentially of an aqueous solution of about 3% by weight of hydrofluoric acid, and from about 20% to about 40% by

weight of a chromium compound selected from the group consisting of chromic acid and its salts, and electroplating said articles in a plating solution.

4. A process for treating the surfaces of articles of titanium and titanium base alloys, including the steps of immersing said articles in a bath consisting essentially of an aqueous solution of about 3% by weight of hydrofluoric acid, and from about 20% to about 40% by weight of sodium dichromate, and electroplating said articles in a plating solution.

5. A process for treating the surfaces of articles of titanium and titanium base alloys, including the steps of immersing said articles in a bath consisting essentially of an aqueous solution of 0.5% to about 20% by weight of hydrofluoric acid, and from about 15% by weight to the saturation point of a chromium compound selected from the group consisting of chromic acid and its salts, maintaining the temperature of said bath at about 180° F. to the boiling point for 10-20 minutes, removing said articles and rinsing the same, and electroplating said articles in a plating solution.

6. A process for treating the surfaces of articles of titanium and titanium base alloys, including the steps, in sequence, of cleaning said articles in an acid etch bath, immersing said articles in a bath consisting essentially of an aqueous solution of 0.5% to about 20% by weight of hydrofluoric acid, and from about 15% by weight to the saturation point of a chromium compound selected from the group consisting of chromic acid and its salts, and electroplating said articles in a plating solution.

7. A process for treating the surfaces of articles of titanium and titanium base alloys, including the steps, in sequence, of cleaning said articles in an acid etch bath, immersing said articles in a bath consisting essentially of an aqueous solution of 0.5% to about 20% by weight of hydrofluoric acid, and from about 15% by weight to the saturation point of sodium dichromate, and electroplating said articles in a plating solution.

8. A process for treating the surfaces of articles of titanium and titanium base alloys, including the steps, in sequence, of cleaning said articles in an acid etch bath, immersing said articles in a bath consisting essentially of an aqueous solution of about 3% by weight of hydrofluoric acid, and from about 20% to about 40% by weight of sodium dichromate, and electroplating said articles in a plating solution.

9. A process for treating the surfaces of articles of titanium and titanium base alloys, including the steps, in sequence, of cleaning said articles in an acid etch bath, immersing said articles in a bath consisting essentially of an aqueous solution of 0.5% to about 20% by weight of hydrofluoric acid, and from about 15% by weight to the saturation point of sodium dichromate, maintaining the temperature of said bath at about 180° F. to the boiling point for 10-20 minutes, removing said articles and rinsing the same, and electroplating said articles in a plating solution.

#### References Cited in the file of this patent

#### UNITED STATES PATENTS

|           |                 |                |
|-----------|-----------------|----------------|
| 1,544,451 | Hambuechen      | June 30, 1925  |
| 1,978,791 | Hale            | Oct. 30, 1934  |
| 2,127,640 | Brown           | Aug. 23, 1938  |
| 2,171,546 | Kapps           | Sept. 5, 1939  |
| 2,311,623 | Blackmun et al. | Feb. 23, 1943  |
| 2,471,909 | Spruance        | May 31, 1949   |
| 2,478,171 | MacPherson      | Aug. 9, 1949   |
| 2,507,956 | Bruno et al.    | May 16, 1950   |
| 2,711,364 | Beach           | June 21, 1955  |
| 2,734,837 | Hands           | Feb. 14, 1956  |
| 2,764,538 | Smart           | Sept. 25, 1956 |

#### OTHER REFERENCES

Handbook on Titanium Metal, 7th ed., August 1, 1953, Titanium Metals Corporation, New York, pp. 92-93.